

## 1

3,097,162

## METHOD FOR CONCENTRATING ALUMINUM SILICATES AND ZIRCON FROM BEACH SAND

Robert E. Baarson, La Grange, and Charles W. Jonaitis, Chicago, Ill., assignors to Armour and Company, Chicago, Ill., a corporation of Delaware

No Drawing. Filed Dec. 2, 1960, Ser. No. 73,231

2 Claims. (Cl. 209—166)

This invention relates to a method for concentrating aluminum silicates and zircon in sand deposits which are usually known as beach sands. More particularly, this invention relates to a method for making a bulk separation of the non-conductive and non-magnetic minerals in beach sands from the quartz.

Beach sands of the type which the present invention is concerned may be found along the sea shore, but are also found in large inland deposits in Florida and elsewhere. These sand beds or deposits are composed principally of quartz, while containing a small proportion of valuable minerals, among them being titanium oxide minerals like ilmenite and rutile, in addition to the heavy minerals such as kyanite-sillimanite, zircon, staurolite and dumortierite. Usually the content of quartz in these sands will be at least 90°, while the content of the various heavy minerals may range from a trace to upwards of 4%.

The most valuable product at present in beach sands is the titanium oxide minerals. These and other conductive and magnet-responsive heavy minerals are recovered from beach sand deposits by complicated and expensive procedures. For example, the steps in one of these processes involves passing the beach sands through a series of spiral concentrators to make a rough separation of the titanium oxide and other heavy minerals from the quartz. Following the rough separation, there are cleaner and recleaner spiral circuits to upgrade the concentrate, and a large amount of the middling material is recycled through these circuits to increase recovery. The titanium minerals in the heavy mineral concentrate are then further separated and concentrated by electrostatic and magnetic separators. The electrostatic separation removes the ilmenite and rutile while induced roll magnets are employed to remove the staurolite and dumortierite.

The resultant non-conductive, non-magnetic reject fractions from this operation contain minerals which are in themselves valuable. The composition of these fractions is roughly 40 to 50% aluminum silicates, also referred to as the kyanite-sillimanite fraction, 20% to 30% zircon, and 25 to 40% quartz. Heretofore, there has been no practical and commercially feasible way of recovering these valuable minerals from the reject beach sand concentrates. It is with these fractions that the present invention is principally concerned.

The problem involved in using such non-conductive non-magnetic ores to obtain an aluminum silicates and zircon product of high grade in economically practical recoveries has heretofore received little attention. The industry has always realized that this discarded material contains valuable heavy minerals but no commercially feasible method has up to now been devised to obtain the minerals in proper grade and recovery. Applicants have solved the problem and have provided through this invention a flotation method which enables the bulk concentration of the valuable aluminum silicate and zircon fractions from the non-conductive, non-magnetic fraction of beach sand concentrates.

It is therefore a general object of this invention to provide a method for concentrating the aluminum silicates and zircon minerals in beach sands, and specifically, to provide a flotation method for accomplishing the concentration of aluminum silicates and zircon from beach sand concentrates from which the titanium oxide minerals have

## 2

been removed. More specifically, it is an object of this invention to provide a floatation method by means of which the aluminum silicates and zircon in such beach sand concentrates can be separated from the quartz. It is still another object of this invention to provide a method for carrying out the bulk separation of aluminum silicates in reject sands concentrates from the quartz and zircon therein, and further, to provide a method for separating the zircon from the quartz without the need for additional quantities of collecting agent. Further objects and advantages will appear as the specification proceeds.

In practicing the present invention, the beach sand fraction from which the titanium oxide minerals have been separated is formed into a floatation feed. The particles of this fraction, as received, range from about —30 to +200 mesh. To the floatation feed is added an amine collector, and a depressant selected from the group consisting of dextrans, gums and starches. The aqueous feed is adjusted to an alkaline pH, and a frother, such as pine oil or cresylic acid, is introduced into the feed. Amine collectors impart some frothing in themselves and for this reason the use of a frothing agent in the process is optional and may be omitted. Employing standard floatation procedures, an aluminum silicates concentrate is obtained in the underflow while a combined zircon and quartz product is recovered in the overflow.

The overflow product may then be re-pulped and worked into a floatation feed to which is added a depressant in the form of a fluorine containing acid. The pH of this feed is adjusted to below about 6.0, preferably about 3.0. A frother, as in the initial floatation operation, may be added. It is generally unnecessary to introduce further quantities of the amine collector. Again employing conventional floatation techniques, a zircon concentrate is obtained in the overflow leaving a tailing consisting primarily of quartz.

Any amine collector can be employed. Preferably, however, the amine floatation agent is a primary amine containing a hydrophobic group of from 6 to 22 carbon atoms. Mixed amines like primary, tallow and soya amines are suitable. Both mono and polyamines may be used. Very satisfactory results are obtained when the amine floatation agent is used in the form of a water-soluble salt thereof, such as an amine acetate or hydrochloride salt. Amine-nitrile blends sold under the trademark Armsfolute, and amines alone, taken up in a frother such as pine oil or an alcohol such as isopropanol, are also effective.

To achieve the outstanding results of the present invention it is only necessary to add small quantities of the collecting agent to the ore. Usually, from about 0.1 to about 4.0 pounds of the agent per ton of ore will be satisfactory, with from 0.3 to about 1.0 pound per ton being preferred.

The pH of the aqueous feed formed from the starting beach sand fraction may be controlled by the addition of minor amounts of such inorganic alkaline reagents as sodium or potassium hydroxide. A pH of from 7.5 to 12 may be used but a range of 8 to 10 is preferred. The important point is to have a sufficient amount of the alkaline reagent present to maintain the pH of the alkaline side.

The depressant employed in bringing about a separation of the aluminum silicates from the zircon and quartz may, as indicated, be selected from the group consisting of dextrans, gums and starches. These agents have the effect of depressing the aluminum silicate fraction of the beach sand permitting the zircon and quartz floatation to be recovered in the overflow.

The fluorine containing acid employed to effect a separation between the zircon and quartz is preferably hydrofluoric acid, although other fluorine containing acids

can be substituted as well as mixtures of hydrofluoric acid and other fluorine containing acids.

The pulp density in the conditioning and flotation circuits may be varied widely. In the conditioning circuit the solids may be as low as 25%. However, 60 to 85% solids is preferred and 70% solids is considered an optimum condition. In the flotation circuit the solids may run as high as 40% and as low as 15%. A 25% pulp density, however, is especially effective for flotation.

The flotation operations described above can be carried out in the usual type of flotation cells provided with means for supplying air to the lower portion of the cells. It is significant that the method of this invention permits a clean separation to be made between all of the aluminum silicates from the zircon and quartz on the one hand and the zircon from the quartz on the other. The separate mineral concentrates can be further upgraded by

#### Metallurgical Results

| Product                  | Weight, grams | Weight, percent | Percent heavy minerals | Percent grade | Percent recovery |
|--------------------------|---------------|-----------------|------------------------|---------------|------------------|
| Aluminum silicates conc. | 266           | 53.2            | 92.50                  | 72.2          | 90.5             |
| Zircon conc.             | 88            | 17.6            | 93.98                  | 84.6          | 61.3             |
| Quartz conc.             | 146           | 29.2            | 10.87                  |               |                  |
| Composite                | 500           |                 |                        |               |                  |

10

#### EXAMPLE II

Preparation of ore ----- As received.  
 Flotation machine ----- Fagergren.  
 15 Water ----- Distilled.  
 Temperature ----- 25° C.

#### Reagents and Conditions

| Point of addition | Conditions      |              |                |                | Reagents, pounds per ton |         |      |          |          |
|-------------------|-----------------|--------------|----------------|----------------|--------------------------|---------|------|----------|----------|
|                   | Time cond.      | Float (min.) | Percent solids | pH             | Starch 3366              | Armac T | NaOH | Pine oil | HF (48%) |
| 1st rougher       | { $\frac{1}{4}$ | 2            | 20             | 9.1 I<br>7.6 F | 3.0                      | 0.12    | 0.8  | 0.17     |          |
| 2nd rougher       | { $\frac{1}{4}$ | 2            |                | 9.3 I<br>7.3 F |                          | 0.2     | 0.04 | 0.17     |          |
| Zircon conc.      | { $\frac{1}{4}$ | 2            |                | 3.0 I<br>3.0 F |                          |         |      | 0.08     | 2.54     |

NOTE.—1st and 2nd roughers filtered and combined in cell for addition of hydrofluoric acid (48%) and subsequent flotation. Starch 3366 obtained from Corn Products. (Unmodified Corn Starch.)

gravity separation, electrostatic or magnetic separation, etc. to give the very high grade required of these minerals. 40 This procedure enables the recovery of 90% or more of the aluminum silicates and zircon contained in the beach sand concentrates.

Whereas these materials were treated as a waste product in normal beach sand operations from which titanium oxide minerals were concentrated the method of this invention now provides a practical and commercially feasible means for recovering valuable products from these waste materials.

This invention is further described in the following 50 specific examples.

#### EXAMPLE I

Preparation of ore ----- As received.  
 Flotation machine ----- Fagergren.  
 Water ----- Distilled.  
 Temperature ----- 25° C.

#### Metallurgical Results

| Product                  | Weight, grams | Weight, percent | Percent heavy minerals | Percent grade | Percent recovery |
|--------------------------|---------------|-----------------|------------------------|---------------|------------------|
| Aluminum silicates conc. | 161           | 32.3            | 98.29                  | 94.9          | 65.0             |
| Zircon conc.             | 208           | 41.6            | 91.61                  | 60.0          | 89.1             |
| Quartz conc.             | 130           | 26.5            | 9.12                   |               |                  |
| Composite                | 499           |                 |                        |               |                  |

45

#### EXAMPLE III

Preparation of ore ----- As received.  
 Flotation machine ----- Fagergren.  
 Water ----- Distilled.  
 55 Temperature ----- 25° C.

#### Reagents and Conditions

| Point of addition | Conditions      |                 |                |                         | Reagents, pounds per ton |         |      |          |          |
|-------------------|-----------------|-----------------|----------------|-------------------------|--------------------------|---------|------|----------|----------|
|                   | Time cond.      | Float (min.)    | Percent solids | pH                      | Dextrin 164              | Armac T | NaOH | Pine oil | HF (48%) |
| 1st rougher       | { $\frac{1}{4}$ | 2               | 20             | 9.0 I<br>7.5 F<br>9.3 I | 2.0                      | 0.1     | 0.8  | 0.17     |          |
| 2nd rougher       | { $\frac{1}{4}$ | 2 $\frac{1}{2}$ |                | 7.4 F<br>2.95 I         |                          | 0.2     | 0.04 | 0.17     |          |
| Zircon conc.      | { $\frac{1}{4}$ | 1 $\frac{1}{2}$ |                | 3.0 F                   |                          |         |      | 0.08     | 2.54     |

<sup>1</sup>I—Initial; F—Final.

NOTE.—1st and 2nd roughers filtered and combined in cell for addition of hydrofluoric acid (48%) and subsequent flotation. Dextrin 164 obtained from Corn Products. Armac T is an acetate salt of tallow amine.

## Reagents and Conditions

| Point of addition | Conditions      |                 |                |                  | Reagents, pounds per ton |         |          |          |       |
|-------------------|-----------------|-----------------|----------------|------------------|--------------------------|---------|----------|----------|-------|
|                   | Time cond.      | Float (min.)    | Percent solids | pH               | Dextrin 164              | Armac T | Pine oil | HF (48%) | NaOH  |
| 1st rougher       | { $\frac{1}{4}$ | 2 $\frac{1}{4}$ | 20             | 7.8 I.<br>6.25 F | 2.0                      | 0.2     | 0.17     | —        | Trace |
| 2nd rougher       | { $\frac{1}{4}$ | 2               | —              | 8.0 I.<br>6.35 F | —                        | 0.2     | 0.17     | —        | Trace |
| Zircon conc       | { $\frac{1}{4}$ | 1 $\frac{1}{2}$ | —              | 3.7 I.<br>3.8 F  | —                        | —       | 0.08     | 1.97     | —     |

NOTE.—1st and 2nd roughers filtered and combined in cell for addition of hydrofluoric acid (48%) and subsequent flotation. A minute amount of caustic was necessary to raise the pH of the roughers.

## Metallurgical Results

| Product                 | Weight, grams | Weight, percent | Percent heavy minerals | Percent grade | Percent recovery |
|-------------------------|---------------|-----------------|------------------------|---------------|------------------|
| Aluminum silicates conc | 153           | 30.5            | 97.69                  | 95.0          | 63.7             |
| Zircon conc             | 246           | 49.1            | 81.71                  | 60.0          | 93.5             |
| Quartz conc             | 102           | 20.4            | 1.06                   | —             | —                |
| Composite               | 501           | —               | —                      | —             | —                |

## EXAMPLE IV

Preparation of ore As received.  
Flotation machine Fagergren.  
Water Distilled.  
Temperature 25° C.

trate. Percent Heavy Minerals essentially is the total heavy mineral grade in each product obtained, with the remainder being quartz. Percent Grade indicates the grade of the mineral being concentrated, taking into account both the quartz and other heavy minerals as contaminants. Percent Recovery represents that portion of the total mineral appearing in the particular product that is considered to be the concentrate.

While in the foregoing specification this invention has been described in relation to a specific embodiment thereof and many details have been set forth for this embodiment, it will be apparent to those skilled in the art that the invention is susceptible to other embodiments and that many of the details set forth herein can be varied widely without departing from the basic concepts of the invention.

## Reagents and Conditions

| Point of addition | Conditions      |                 |                |                 | Reagents, pounds per ton |           |      |          |          |
|-------------------|-----------------|-----------------|----------------|-----------------|--------------------------|-----------|------|----------|----------|
|                   | Time cond.      | Float (min.)    | Percent solids | pH              | Dextrin 164              | Duo-mac C | NaOH | Pine oil | HF (48%) |
| 1st rougher       | { $\frac{1}{4}$ | 2 $\frac{1}{4}$ | 20             | 9.1 I.<br>7.6 F | 2.0                      | 0.1       | 0.8  | 0.17     | —        |
| 2nd rougher       | { $\frac{1}{4}$ | 2               | —              | 9.2 I.<br>7.4 F | —                        | 0.2       | 0.04 | 0.17     | —        |
| Zircon conc       | { $\frac{1}{4}$ | 1 $\frac{1}{2}$ | —              | 3.0 I.<br>3.0 F | —                        | —         | —    | 2.54     | —        |

NOTE.—1st and 2nd roughers filtered and combined in cell for addition of hydrofluoric acid (48%) and subsequent flotation. Dextrin 164 obtained from Corn Products. Duomac C is a diacetate salt of a coco diamine.

## Metallurgical Results

| Product                 | Weight, grams | Weight, percent | Percent heavy minerals | Percent grade | Percent recovery |
|-------------------------|---------------|-----------------|------------------------|---------------|------------------|
| Aluminum silicates conc | 174           | 34.8            | 96.23                  | 95            | 69.0             |
| Zircon conc             | 192           | 38.3            | 91.34                  | 60            | 88.5             |
| Quartz conc             | 135           | 26.9            | 4.91                   | —             | —                |
| Composite               | 501           | —               | —                      | —             | —                |

## REMARKS

The ore in the tests conducted was the resultant non-conductor, non-magnetic product from electrostatic separation and separation over induced roll magnets. The electrostatic separation removed the ilmenite and rutile while the induced roll magnets removed the staurolite and dumortierite leaving an aluminum silicates-zircon-quartz fraction. This fraction had an approximate composition of 45% aluminum silicates, 25% zircon, and 30% quartz. Compositions on this and subsequent concentrates were obtained by petrographic analysis. Heavy mineral analysis was obtained by heavy media separation.

The analyses indicate an upgrading of minerals in both the aluminum silicates concentrate and the zircon concen-

## 50 We claim:

1. In a process for the concentration of quartz, aluminum silicate and zircon from a non-conductive, non-magnetic fraction of beach sand concentrate, comprising the steps of floating a zircon and quartz fraction from the aluminum silicates in the sand in an aqueous solution containing an amine collector and a depressant selected from the group consisting of dextrins, gums and starches, said aqueous solution being at a pH of from about 7.5 to about 12, and then floating the zircon from the quartz of said zircon-quartz fraction in the presence of a fluorine-containing acid and at a pH from about 6.0 to about 2.0.

2. In a process for the concentration of quartz, aluminum silicate and zircon from a non-conductive, non-magnetic fraction of beach sand concentrate, comprising the steps of floating a zircon and quartz, fraction from the aluminum silicates in the sand in an aqueous solution at a pH of about 8.0 containing an amine collector and a depressant selected from the group consisting of dextrins, gums and starches, said amine collector having at least one hydrophobic group of from 6 to 22 carbon atoms, and then floating the zircon from the quartz of said zircon-quartz fraction, without adding more of the collecting agent in the presence of a fluorine-containing acid and at a pH of about 3.0.

References Cited in the file of this patent  
UNITED STATES PATENTS

2,177,985 Harris ----- Oct. 31, 1939  
2,205,503 Trotter ----- June 25, 1940  
2,341,046 Kirby ----- Oct. 9, 1940

2,792,940 Baarson ----- May 21, 1957  
2,970,688 Uhland ----- Feb. 7, 1961

## OTHER REFERENCES

Gaudin: Flotation, page 500 (Sillimanite and Kyanite),  
Second Edition, McGraw-Hill, 1957.